

(No Model.)

C. C. SCAIFE.

3 Sheets—Sheet 1.

METHOD OF MAKING ELEVATOR BUCKETS.

No. 349,754.

Patented Sept. 28, 1886.

Fig. 3.



Fig. 4.



Witnesses.

M. T. Corwin

H. L. Gill.

Fig. 5.



Fig. 2.



Inventor:  
Charles C. Scsafe  
by his atty  
Bakewell & Kent

(No Model.)

C. C. SCAIFE.

3 Sheets—Sheet 2.

METHOD OF MAKING ELEVATOR BUCKETS.

No. 349,754.

Patented Sept. 28, 1886.

Fig. 8.



Fig. 6.



Fig. 9.



Fig. 7.



Witnesses.

H. A. Corwin  
H. L. Gill.

Inventor.

Charles C. Scife  
by his attys  
Bakerwell & Kester

(No Model.)

3 Sheets—Sheet 3.

C. C. SCAIFE.

METHOD OF MAKING ELEVATOR BUCKETS.

No. 349,754.

Patented Sept. 28, 1886.

Fig. 11.



Fig. 10.



Fig. 13.



Fig. 14.  $\alpha'$



Fig. 15.  $\alpha'$



Fig. 12.



Witnesses.

W. D. Cowrie  
H. L. Gill

Inventor:  
Charles C. Scaife  
by his attys  
Bakewell & Steers

# UNITED STATES PATENT OFFICE.

CHARLES C. SCAIFE, OF ALLEGHENY CITY, PENNSYLVANIA.

## METHOD OF MAKING ELEVATOR-BUCKETS.

SPECIFICATION forming part of Letters Patent No. 349,754, dated September 23, 1886.

Application filed June 17, 1886. Serial No. 205,510. (No model.)

*To all whom it may concern:*

Be it known that I, CHARLES C. SCAIFE, of Allegheny City, in the county of Allegheny and State of Pennsylvania, have invented a new and useful Improvement in the Manufacture of Elevator-Buckets; and I do hereby declare the following to be a full, clear, and exact description thereof.

It is very desirable to make elevator-buckets of a single piece of metal, so that they shall be free from rivets and seams, and present smooth unbroken surfaces, because the discharge of the contents is thereby facilitated, the bucket is not liable to become clogged, and is not liable to catch upon or injure the trough or conductor in which it moves. Elevator-buckets having these qualities have been formed by casting out of malleable iron; but such buckets are extremely heavy and expensive. Consequently their use has been limited. It has been suggested to make such buckets out of a single piece of sheet metal by striking it up by any suitable dies, but, so far as I can ascertain, such a bucket was never successfully made until produced by me in the use of the method I am about to explain. This was owing to the difficulty of giving the proper shape and depth to the cup of metal, the strain of the stamping operation being too great for the strength and tenacity of the material. After long-continued experiments I discovered my present method of making these buckets, and have had the same in extensive and successful practical operation for some time past.

To enable others skilled in the art to make and use my invention, I will now describe it by reference to the accompanying drawings, in which—

Figure 1 is a plan view of the die and plunger with which the first step of the operation is performed. Figs. 2 and 3 are vertical sections on the lines A A and B B of Fig. 1. Fig. 4 is a view of the blank. Fig. 5 is a view of the same after undergoing the first step of the operation. Fig. 6 is a longitudinal section of the second die and plunger. Fig. 7 is a cross-section of the product of the second die. Fig. 8 is a longitudinal view of the third die and plunger. Fig. 9 is a cross-section of the product of the third die. Figs. 10 and 11 are longitudinal and cross sections of the fourth die

and plunger. Fig. 12 is a view of the product of the fourth die. Fig. 13 is a view of the trimming-dies. Fig. 14 is a view of the trimmed blank. Fig. 15 is a view of the finished bucket.

55

Like letters of reference indicate like parts in each.

In practising this invention I take a blank, *a*, Fig. 4, of steel or iron, and place the same cold upon the surface of the die *b*. (Shown in Figs. 2 and 3.) This die *b* is secured to the bed-plate of a drop-press of the ordinary construction, which press is provided with a clamping-ring, *c*, which descends upon and clamps the edge or edges of the blank *a* over the cavity *b'* of the die *b*. The plunger *d* then descends through the clamping-ring and forces the middle portion of the blank *a* down into the cavity *b'*, producing a shallow cup-shaped blank, such as is shown at *a'*, Fig. 5. The effect of this stamping operation upon the metal blank is to render it so hard that I find it desirable to anneal it, which may be done by placing it in a heating-furnace and heating it up to a cherry red, and then permitting it to cool in the open air. This blank is then submitted to the operation of the die and plunger *e f*, (shown in Fig. 6,) which, being of greater depth and smaller diameter, have the effect of reducing the diameter and increasing the depth of the cup and producing a blank, *a''*, such as is shown in Fig. 7. The process of annealing is then repeated, and the blank *a''*, after becoming cold, is submitted to the operation of the die *h* and plunger *i*, (shown in Fig. 8,) which, being less in diameter and greater in depth, 75 reduce the diameter and increase the depth of the blank, as shown at *a'''*, Fig. 9. The blank is then heated; but instead of being permitted to cool it is taken directly from the heating-furnace and put upon the die *k*, (shown in Figs. 10 and 11,) where the final shape is given to the cup by the plunger *m*, as shown at *a''''* in Fig. 12. This bucket has a round bottom, flaring sides, and straight ends, the ends being slightly divergent. After this step the blank *a''''* is placed in a die, *n*, (shown in Fig. 13,) and is there subjected to the action of the shear or plunger *o*, which trims off the flange, except on the rear side of the cup, as shown at *a'''''* in Fig. 14, where the flange is merely trimmed straight, so that it may be laid down against

75

80

85

90

95

100

the side of the cup, as shown in Fig. 15, to constitute a re-enforcement or extra thickness of the metal at that point where it is riveted or bolted to the belt. This method enables the material to stand the severe stamping operation without fracture. It is only by performing the last step of the operation upon the blank in a heated condition that I am able to give it its proper shape. The wide mouth, narrow bottom, and great depth make it an extremely difficult article to make, and I know of no other practical way of doing it except the one I have described. It is strong, light, of proper shape to discharge its contents properly, and very durable.

What I claim as my invention, and desire to secure by Letters Patent, is—

The method of making elevator-buckets, which consists in striking up a blank of cold plate metal into a cup shape by a series of operations in dies increasing in depth and decreasing in width in regular order, whereby the cup is increased in depth and decreased in diameter at each step, annealing the blank during the operation, and finally shaping it hot in a suitably-shaped die, substantially as and for the purposes described.

In testimony whereof I have hereunto set my hand this 12th day of June, A. D. 1886.

CHARLES C. SCAIFE.

Witnesses:

W. B. CORWIN,  
JNO. K. SMITH.